

# UNITED STATES PATENT OFFICE.

F. DE CAMPOLORO, OF NEW YORK, N. Y.

## IMPROVEMENT IN THE MANUFACTURE OF PAPER-PULP.

Specification forming part of Letters Patent No. 29,471, dated August 7, 1860.

*To all whom it may concern:*

Be it known that I, F. DE CAMPOLORO, a native of the Empire of France, at present residing in the city, county, and State of New York, have invented a new and Improved Mode of Producing Pulp for the Manufacture Paper, &c.; and I do hereby declare that the following is a full, clear, and exact description of the same:

My invention consists in the employment for the purpose of producing pulp for the manufacture of paper, &c., of the cobs of Indian corn or maize, either alone or with the husks.

To enable those skilled in the art to make and use my invention, I will proceed to describe it.

The large quantity of corn in this and other countries and the qualities of the leaves and stalks of the same have induced manufacturers and inventors to make manifold experiments for the purpose of finding out the proper means to use said parts of the corn for paper-pulp, and they have succeeded as far as the inferior sorts of paper are concerned; but it has not been proposed in any case to use the cobs of corn; neither have former experiments with other parts of this plant been successful in producing white paper. The cobs in themselves are generally so white that the same, when boiled and mashed up in a proper vessel, form a pulp of sufficient whiteness to form white paper without previously bleaching the pulp; but if the cobs, together with the husks, are used, the pulp produced from the same has

first to be bleached before it can be used for the manufacture of white paper.

The bleaching, where it is necessary, I accomplish in the ordinary manner by the means of chlorine, or by the employment of hypochloride of potash or of soda, either with or without the application of heat, and the pulp thus produced can be employed for the purpose of manufacturing perfectly white paper in the ordinary manner.

By these means I am enabled to produce a cheap paper of good qualities, and the material for the pulp will not likely become scarce, since I make use of those parts of the corn which are generally considered of very little or no value for any other purpose.

I am aware that the stalks and leaves of corn have been used before for the purpose of producing pulp for paper. Those I do not claim; neither do I claim the employment for this purpose of the husks or covering-leaves of the ears, such having been proposed by Mr. D. Harcourt in his English patent of 1838; but

What I do claim as new, and desire to secure by Letters Patent, is—

The employment of the cobs of Indian corn, either alone or with the husks, substantially as herein described, for the purpose of producing pulp for paper.

F. DE CAMPOLORO.

Witnesses:

W. HAUFF,  
J. F. BUCKLEY.